

July 21, 1953

E. L. BAXTER

2,646,366

BACKING PAPER FOR ROLL PHOTOGRAPHIC FILM

Filed Dec. 8, 1951

**Fig. 1**



**Fig. 2**



**Ernest L. Baxter**  
INVENTOR.

BY Daniel J. Mayne,  
Walter O. Hoddon

ATTORNEYS

## UNITED STATES PATENT OFFICE

2,646,366

BACKING PAPER FOR ROLL  
PHOTOGRAPHIC FILMErnest L. Baxter, Rochester, N. Y., assignor to  
Eastman Kodak Company, Rochester, N. Y., a  
corporation of New Jersey

Application December 8, 1951, Serial No. 260,714

2 Claims. (Cl. 117—14)

1

This invention relates to improvements in backing paper for roll photographic film, and more particularly relates to a backing paper with protective light-colored and opaquing coatings thereon, which has appreciably less overall thickness than conventional backing papers, and which is superior in opaqueness and equal in other respects to presently employed duplex backing paper.

The backing paper of this invention is an improvement over that described and claimed in my copending patent application Ser. No. 187,124, filed September 27, 1950.

As is well understood, a photographic roll film cartridge generally comprises a flanged spool upon which is wound a long strip of backing paper to which before winding has been attached a strip of light sensitive photographic film. The ends of the backing paper are positioned to extend beyond the ends of the film and constitute light protective leader and trailer strips for the film which is interwound with the backing paper and, therefore, separates adjacent convolutions of the film.

In a commonly available roll film cartridge, the film is attached to the black side of a duplex backing paper, the side of the backing paper opposite that contacting the film is differently colored and carries various printed symbols such as the number of the exposed areas, warning marks, and advertising matter, over which is coated a protective layer intended to protect the sensitive emulsion from the paper and ink employed in printing when the film and paper are interwound in close contact. It has been the practice to depend somewhat on the paper itself to prevent the transmission of light. To assure opaqueness, backing paper presently employed for roll films generally consists of a duplex paper with one side being black and the other side colored with a characteristic identifying color. The paper may be made by means of a Fourdinier paper machine and a cylinder paper machine. The two sheets are brought together wet under the first press and thus form a single composite sheet of backing paper.

Duplex backing paper has certain definite specifications that must be met. The black side must be opaque and free from pinholes. The lighter colored side should be uniform in color and appearance and should not permit any of the black on the opposite side to be visible through the paper. The diameter of the finished spool of roll film, and, therefore, the number of exposures, is dependent on the overall thickness

2

of the backing paper and the film, so thickness of the paper itself must be limited. The required strength of the paper which is important both in the camera and in processing, also limits the thinness of the paper. Either black numerals on a white paper or white numerals on a black paper give the greatest contrast, but neither paper is very pleasing to the eye. Lighter colored backgrounds such as shades of red, green, yellow and blue are most desirable from an appearance standpoint.

It does not appear possible for a paper mill to make a duplex backing paper thinner than those in current use, which will fulfill the necessary requirements of such a paper. In order that the sheet may be photographically opaque, a certain minimum weight and thickness of black is required. The lighter the shade and color of the other side, the greater is the weight and thickness of paper required to hide the black side and to give the light colored side a uniform appearance. The present invention, however, provides a thinner backing paper which does not have a duplex structure but which has superior characteristics.

An object, therefore, of the present invention is to provide a backing paper comprising a single sheet of paper, as contrasted to a duplex paper, which has a strength at least equal to the thinnest duplex papers now produced.

Another object of the invention is to provide a single sheet coated backing paper which is not thinner than present duplex paper, but has an opaqueness superior to duplex backing papers.

Another object of the present invention is to provide a thin single sheet backing paper, the opacity of which is dependent primarily on the chemical coatings on the paper rather than the paper structure itself.

Still another object is to provide a backing paper having an improvement in overall thinness so that extra film exposures are permitted without increasing the diameter of the roll beyond that of the same type of presently employed roll film.

Yet another object is to provide a backing paper comprising a single sheet of paper with black opaquing coatings thereon which are more flexible than those black coatings on the backing papers described in my copending application Ser. No. 187,124, filed September 27, 1950.

In accordance with the invention these and other objects are attained by employing as the paper strip in the backing paper a single sheet, as contrasted to a duplex paper, which has been

supercalendered to a thickness appreciably less than commonly employed duplex papers. By itself this paper is so thin that it transmits sufficient actinic light to cause film exposure. This single paper is then coated on one side with one or more black opaque coatings and on the other side by a composite coating of lighter colored composition. The paper may then be printed on the lighter colored side and, if so printed, the printed side is given a protective overcoating to protect the film emulsion from the printing inks. The various coatings may be applied in proper sequence by a rotogravure process or by other suitable coating processes. The coatings may be suitably dried between applications.

The paper preferably employed as the base of the backing paper structure is a 15-pound per 1000 sq. ft. paper made of a purified fiber or of unpurified fiber such as unbleached kraft paper which is conditioned to 4-12% moisture content and supercalendered to a thickness of 0.0025 to 0.0030 inch. This thin paper is then coated on one side with a plurality of black coatings. The opposite side of this thin paper is coated with a yellow coating. The composition of the black and yellow coating is described hereinafter. The thus coated paper is printed on the yellow side with suitable legends and overcoated with a protective coating of a prolamine to protect the film emulsion from the printing inks when the film and backing paper is rolled onto the film spool.

The following colored coating compositions are preferred for use in preparing a backing paper in accordance with my present invention:

*Initial black coatings*

|                   | Pounds |
|-------------------|--------|
| Polyvinyl acetate | 15     |
| Carbon black      | 10     |
| Water             | 18.6   |
| Methyl alcohol    | 56.4   |

*Final black coating*

|               | Pounds |
|---------------|--------|
| Zein          | 20     |
| Paris black   | 10     |
| Water         | 4      |
| Alcohol:      |        |
| Ethyl alcohol | 66.6   |
| Methyl        | 3.6    |
| Water         | 10.0   |

*Yellow coating*

|                       | Pounds |
|-----------------------|--------|
| Zein                  | 20     |
| Medium chrome yellow  | 10     |
| Light orange (chrome) | 5      |
| Titanox               | 15     |
| Isopropyl alcohol     | 64     |
| Water                 | 16     |

In the above formulas, titanox represents a finely divided titanium pigment; medium chrome yellow is a finely divided metal chromate pigment; light orange is a finely divided metal chromate pigment, and the carbon black pigments are similarly finely divided. Zein is employed as the binder in the yellow and final black coating since it will not fog or desensitize the photographic emulsion of the film.

A suitable rotogravure process for applying these coatings to the paper base of the backing paper is described in U. S. Patent 2,218,249 of October 15, 1940. The various applications are

made continuously and each coating is dried before the next is applied. The coating is applied to the paper by the intaglio roll which is rotatably mounted in a pan containing the coating solution. The surface of the roll is embossed providing a plurality of very minute cups which carry the solution, the excess solution being removed from the roll by a doctor blade. The solution in these various cups is then transferred or applied uniformly to the strip by pressing the strip against the cups by means of a rubber pressure roll over which the strip is fed. Each of these deposits after being placed on the paper is merged into a continuous layer by means of a smoothing bar to provide a uniform coating over the entire paper surface. Each coating is preferably dried in heated air having a relative humidity of 6% at 170° F. before applying a second coating.

Suitable ink compositions for printing indicia by rotogravure processes on the backing paper are disclosed in my Patent Re. 21,268 of November 21, 1939. These inks comprise suitable coloring materials in a prolamine binder such as zein. Other suitable coatings for such backing papers are disclosed in my Patent 2,262,986 of November 18, 1941.

The invention will be further understood by reference to the drawings in which Fig. 1 represents a greatly enlarged cross-section of backing paper made in accordance with my present invention, and Fig. 2 shows the backing paper and photographic film wound on the roll with the film and paper separated at one end for purpose of illustration.

Referring to Fig. 1, a strip of unbleached kraft paper is shown at 10 having a coating 11 of a layer of carbon black in a polyvinyl acetate binder thereon which is overcoated with a layer of carbon black in a zein binder. On the opposite side of the paper 10, there is the yellow coating 13 comprising orange and yellow pigments as well as titanium dioxide pigments. The printed indicia is shown at 16 overcoated with a protective zein coating 15. Such a protective coating is described in my Patent 2,262,987 of November 18, 1941.

Referring to Fig. 2, a film cartridge 20 is shown partly open in which the backing paper of the present invention is employed. This figure shows the relation of the backing paper surfaces 11 and 15 in respect to the film 21 when assembled on the spool. The emulsion side of the film is shown at 23 and the pellid side at 22.

I have found that by employing an initial coating of carbon black in polyvinyl acetate, which is overcoated with carbon black in zein on the black side of the paper, the resulting backing paper structure has considerable improvement in respect to flexibility of the black side without loss of resistance to scratching and abrasion. In this respect the backing paper of the present invention is superior to that described and claimed in my copending application Ser. No. 187,124, supra. The polyvinyl acetate binder coating is less brittle than a zein coating of a corresponding thickness. However, with the thickness of the zein coating heretofore required reduced by the polyvinyl acetate coating, the remaining zein overcoating is thin and flexible enough to withstand the bending of the backing paper while at the same time providing an abrasion resisting layer over the softer polyvinyl acetate.

While the preferred coating compositions are described above, satisfactory backing papers may

be made by employing the various coating materials in the following ranges:

| Compositions      | Preferred Range |
|-------------------|-----------------|
| Zein              | 7 to 25.        |
| Polyvinyl acetate | 5 to 25.        |
| Black pigment     | 1 to 15.        |
| White pigment     | 15 to 45.       |
| Yellow pigment    | 15 to 45.       |
| Solvent:          |                 |
| Water             | 5 to 20.        |
| Alcohol           | 95 to 80.       |

| Other solvent compositions useful with zein: | Per cent |
|----------------------------------------------|----------|
| Ethyl alcohol                                | 55       |
| Ethylene chloride                            | 45       |
| Ethyl alcohol 95%                            | 80       |
| Methyl ethyl ketone                          | 20       |

Other useful pigments are, for example, Hansa Yellow, Fast Pigment Yellow and any carbon black of suitable dispersion.

Other pigments which are inert to photographic emulsions may be employed. In fact, any choice of pigments of suitable size for this invention is limited only by the requirement that they be without detrimental effect on the photographic film.

#### Thickness of coating

Black coating composition is applied in four coatings to give a total of 12 lbs. of solution per 1000 sq. foot for satisfactory opacity.

Light pigment composition is applied in the amount of 4 1/4 lbs. per sq. foot to give satisfactory uniformity of color.

Any other type of paper may be employed if it has good strength at least comparable to the present duplex paper. A rag paper, for example, is suitable but, of course, more expensive than kraft paper.

#### Comparison of duplex and kraft tear strength

|                                                        | Elmendorf Tear |            | Schopper Folds |        |
|--------------------------------------------------------|----------------|------------|----------------|--------|
|                                                        | Along          | Across     | Along          | Across |
| Typical Duplex Paper                                   | Gms.<br>70     | Gms.<br>84 | 410            | 28     |
| Tan Kraft Paper (as employed in the present invention) | 65             | 75         | 475            | 100    |

Preferably the average tear strength of a suitable paper should be at least 50 gms. as determined by the Elmendorf tear test. This tear test is described in Paper Trade Journal for June 18, 1942 as Tappi Standard T414 M40.

While polyvinyl acetate is the preferred binder for the opaquing coating, other binders may be employed in its place such as vinylidene-vinyl chloride polymers such as "Geon" or "Saran" and the butadiene-styrene type polymers such as Dow "Latex." These polymers may be applied as latices as well as from solvent solutions. The following composition illustrates such a suitable alternative opaquing medium

|             | Pounds |
|-------------|--------|
| Saran latex | 133    |
| Aquablak B  | 100    |
| Water       | 29     |

The Saran latex contains 52.5% solids and the Aquablak B is a 35% dispersion of carbon black in water.

While, as indicated above, tan kraft paper is particularly suited for employment in my invention, certain other types of paper could be employed instead, such as unbleached sulfate paper colored with a suitable dye such as Stilbene yellow in which a small amount of filler such as TiO<sub>2</sub> is added to give body and density or opacity to the paper.

These papers comprising the base of the backing paper are of a weight that can be supercalendered to a thinness that the paper itself plus the coatings thereon does not exceed a maximum thickness of 0.0040 inch. A 15-pound per M sq. ft. paper has been found satisfactory.

The opacity of roll film backing paper is tested in the following manner.

A sheet of the backing paper under test is placed over a sheet of highly sensitive film, such as Super XX Panchromatic Film with the black side of the backing paper in contact with the back of the film, duplicating its position on roll film. An orange-red filter of the type employed in camera back windows is placed over the opposite side of the backing paper and the assembly is placed in a printing frame. The test material is exposed to a light intensity of 5000 feet candles for ten minutes. The film is then processed in the usual way and examined for the presence of specks of developed silver. A satisfactory backing paper should show no visible silver image.

I have found that my improved backing paper has many advantageous features not possessed by duplex papers which it may replace. The strength and other physical properties of the paper employed as the base of the backing paper is at least equal to the strength of the thinner duplex papers now available to the trade. The overall thickness can be made as low as 0.0032 up to 0.0040 inch thus permitting extra exposures to be added to present rolls of film without increasing the diameter beyond that of films now in use. The opaqueness, even though the overall thickness is less than backing papers now available in the trade, is better than such backing papers. The backing paper made in accordance with my invention requires the least amount of coating materials, both black and colored, of any of the methods described or known in the trade. The uniformly light colored side gives maximum contrast with the legends printed thereon. Also less clock springing of freshly rolled film is experienced with this paper than with the thicker duplex paper. These advantages plus the advantages of applying the coatings by rotogravure methods, which are fast, accurate and efficient, emphasizes the importance of my present invention in this art.

What I claim and desire to secure by Letters Patent of the United States is:

1. Photographic backing paper having an overall thickness less than 0.0040 inch comprising a single sheet of kraft paper, as contrasted to a multiple sheet of duplex paper, of a thickness of approximately 0.0026 inch which will permit passage of substantial amounts of actinic light, having on one side an opaquing coating comprising carbon black in a polyvinyl acetate binder which is overcoated with a second opaquing coating comprising carbon black in a zein binder, a lighter colored pigmented coating on the opposite surface of the paper comprising a yellow pigment in a zein binder, printing on said lighter colored coating, and a clear zein protective coating thereover, the complete backing paper being sufficiently opaque to prevent actinic light from passing therethrough.

2. Photographic backing paper having an overall thickness less than 0.0040 inch comprising a single sheet of tan kraft paper, as contrasted to a multiple sheet of duplex paper, of a thickness of approximately 0.0026 inch which will permit passage of substantial amounts of actinic light, having on one side an opaques coating comprising carbon black in a polyvinyl acetate binder which is overcoated with a second opaques coating comprising carbon black in a zein binder, a lighter colored pigmented coating on the opposite surface of the paper comprising a yellow pigment in a zein binder, printing on said lighter colored coating and a clear zein protective coating thereover, the complete backing paper 15

being sufficiently opaque to prevent actinic light rays from passage therethrough.

ERNEST L. BAXTER.

References Cited in the file of this patent

UNITED STATES PATENTS

| Number    | Name            | Date          |
|-----------|-----------------|---------------|
| 1,481,529 | Baltz et al.    | Jan. 22, 1924 |
| 1,614,490 | Poorman         | Jan. 18, 1927 |
| 1,820,168 | Vehl et al.     | Aug. 25, 1931 |
| 1,954,333 | Sheppard et al. | Apr. 10, 1934 |
| 2,157,206 | Hinman          | May 9, 1939   |